



US005327621A

## United States Patent [19]

Yasui et al.

[11] Patent Number: 5,327,621

[45] Date of Patent: Jul. 12, 1994

## [54] METHOD OF PRODUCING FABRIC REINFORCING MATRIX FOR COMPOSITES

[75] Inventors: Yoshiharu Yasui; Meiji Anahara; Fujio Hori; Junji Takeuchi, all of Kariya, Japan

[73] Assignee: Kabushiki Kaisha Toyoda Jidoshokki Seisakusho, Kariya, Japan

[21] Appl. No.: 34,534

[22] Filed: Mar. 19, 1993

## [30] Foreign Application Priority Data

Mar. 23, 1992 [JP] Japan 4-065158  
Mar. 23, 1992 [JP] Japan 4-065159[51] Int. Cl.<sup>5</sup> D03D 13/00

[52] U.S. Cl. 28/149; 139/11; 139/DIG. 1; 139/430; 28/151; 428/225; 428/257

[58] Field of Search 428/225, 257; 139/430, 139/DIG. 1, 384 R, 34, 11; 112/80.1; 156/393, 148, 163, 164; 28/140, 149, 151

## [56] References Cited

## U.S. PATENT DOCUMENTS

4,725,485 2/1988 Hirokawa 139/DIG. 1 X  
5,121,530 6/1992 Sakatami et al. 28/140 X  
5,211,967 5/1993 Yasui et al. 139/DIG. 1 X

5,224,519 7/1993 Farley 139/DIG. 1 X

## FOREIGN PATENT DOCUMENTS

61-30059 7/1986 Japan  
63-42955 2/1988 JapanPrimary Examiner—Andrew M. Falik  
Attorney, Agent, or Firm—Brooks Haidt Haffner & Delahunty

## [57] ABSTRACT

A reinforcing matrix is produced using a plurality of regulating members (pins) removably arranged in rows in a predetermined direction on a base. Yarns are woven between the pins on the base repeatedly looping back and forth between spaced apart positions to form a yarn lamination consisting of a plurality of yarn layers over the base. The yarns forming the yarn layers are arranged in at least two directions. Thereafter the yarn lamination is removed from the base together with the pins. Then the pins are replaced sequentially in rows arranged in the predetermined direction with separate vertical yarns which are inserted into the yarn lamination so as to form loops. A selvage thread is inserted in the predetermined direction through the loops of the vertical yarns.

9 Claims, 15 Drawing Sheets



FIG. 1



FIG. 2



FIG. 3



FIG. 4



FIG. 5



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19



FIG. 20



FIG. 21



FIG. 22



FIG. 23



FIG. 24



FIG. 25



FIG. 26



FIG. 27



FIG. 28



FIG. 29 (Prior Art)

FIG. 30  
(Prior Art)

## METHOD OF PRODUCING FABRIC REINFORCING MATRIX FOR COMPOSITES

### BACKGROUND OF THE INVENTION

#### 1. Field of the Invention

The present invention relates generally to three dimensional fabrics, and more particularly, it relates to a method of producing a fabric reinforcing matrix for composites.

#### 2. Description of the Related Art

Fabric reinforcing composites are commonly used as light structural materials. A three-dimensional fabric is conventionally used as a reinforcing matrix for a composite. A three-dimensional fabric generally includes three kinds of threads or yarns respectively extending along the X, Y and Z directions. Composites having such a three-dimensional fabric as a frame member, are expected to be widely used as structural materials for rockets, aircraft, automobiles, marine vessels and buildings. The frame member is impregnated with a resin or other inorganic substances. The use of five-axis three-dimensional fabrics, having yarns that are angularly arranged with respect to the longitudinal direction, is proposed. These yarns are provided in addition to the yarns extending along the X, Y and Z directions.

An exemplary method of producing a three-dimensional fiber structure is to laminate a plurality of yarn layers, each formed by arranging lines of yarn repeatedly looped back at both ends, and to interconnect these yarn layers by the lines of yarn running in the thickness (vertical) direction. Such a method is disclosed in Japanese Unexamined Patent Publication No. Sho 63-42955. As shown in FIG. 29, of the present application, this Japanese publication describes apparatus that utilizes a plurality of yarn guide pipes 32 that are placed upright at predetermined pitches on a base plate 31.

Plate-like separators 33 are placed in parallel between the yarn guide pipes 32. A plate-like spacer 34 lies on, and extends perpendicularly to the separators 33. The lines of the first endless yarn Y1 are looped back and engage with the yarn guide pipes 32 located at the peripheral portions of the base plate 31. The lines of the first endless yarn Y1 also weave between the yarn guide pipes 32 in a direction perpendicular to the direction of arrangement of the spacer 34, yielding a yarn layer.

The lines of the first endless yarn Y1 are arranged on the yarn layer and are looped back in a direction perpendicular to the direction of arrangement of the first endless yarn. The arrangement of the first endless yarn Y1 is repeated in the same manner to provide a lamination of a predetermined number of yarn layers, thus yielding a yarn lamination. Next, a spacer 34 is placed on the yarn lamination in the same manner as described above. The yarn lamination is then tightened by the spacers 34 from the top and bottom directions. Then, the yarn guide pipes 32 are replaced with the lines of the second endless yarn Y2, for completing a reinforcing matrix for the composite.

The yarn guide pipes 32 are replaced with the lines of the second endless yarn Y2 in the following manner. First, the separators 33 are removed in order, and the yarn guide pipes 32 are pulled up in succession to the vicinity of the lower spacer 34. Then, the second endless yarn Y2 is bent in a loop (L), and is hooked on a yarn guide 35, which in turn, is inserted into the associated yarn guide pipe 32. Then, the yarn guide pipe 32 is pulled up so that the loop L comes out on the top of the

lamination of the first endless yarn Y1. In this condition, the loop L is removed from the yarn guide pipe 32 and the third endless yarn Y3 is inserted as a tacking yarn through the loop L. Then, the second endless yarn Y2 is pulled down to tighten the yarn lamination. The foregoing steps are repeated each of the yarn guide pipes 32, to complete the replacement of the yarn guide pipes 32 with the lines of the second endless yarn Y2.

In the above method, the yarn lamination is tightened by the cooperation of the lines of the second endless yarn Y2 for coupling the yarn lamination, and the lines of the third endless yarn Y3, which are inserted through the loops L of the endless yarn Y2. The direction of arrangement of the lines of the second endless yarn Y2 on the opposite surface of the yarn lamination to the one where the lines of the third endless yarn Y3 are arranged, is the same as the direction of arrangement of the third endless yarn Y3.

Accordingly, the yarn lamination is firmly tightened at those portions where the lines of the second endless yarn Y2 face the lines of the third endless yarn Y3. As a result, the portions between the tightened portions will rise, causing the yarn lamination to undulate. In other words, the yarn lamination does not have a uniform thickness. This not only causes a periodic variation in the fabric filling factor, but also shortens the length of the reinforcing matrix along the direction perpendicular to the direction of arrangement of the lines of the third endless yarn Y3. Therefore, the intended three-dimensional fiber structure will not be obtained.

In impregnating such a three-dimensional fiber structure with resin, if this structure were not simultaneously pressed and stretched in the direction perpendicular to the undulation, the variation in the fabric filling factor is transmitted directly to the composite and the final product.

In order to provide a large reinforcing matrix, more than ten thousand yarn guide pipes 32 might be needed. Consequently, it would be difficult to replace the yarn guide pipes 32 one by one, with a single second endless yarn Y2.

Further, in the above method, the yarn guide pipes 32 serve as means through which the lines of the second endless yarn Y2 are inserted, and the second endless yarn Y2 is inserted into the yarn lamination at the same time as the associated yarn guide pipe 32 is removed. This method however requires that the yarn guide pipes 32 be pulled from the opposite side to the inserting side of the yarn guide 35. This will not cause any problem when the reinforcing matrix for composite is of a flat type, but will be inconvenient when the reinforcing matrix is U shaped, box shaped, or with narrow spaces between the opposite faces. This is because when the yarn guide pipe 32 is driven out from one side toward the opposite side, the yarn guide pipe 32 might encounter the opposite surface and might not be removed. Further, in pulling the yarn guide pipe 32 in the direction away from the opposite surface, it would be troublesome to insert the yarn guide 35 with the second endless yarn Y2 hooked thereon, into the associated yarn guide pipe 32.

Japanese Patent Publication Sho 61-30059 discloses a method of sewing a plurality of laminations of two-dimensional yarn layers with a sewing machine to produce a three-dimensional fiber structure. The sewing machine used in this method is equipped with an auxil-

iary needle 37 in addition to a sewing needle 36, as shown in FIG. 30 at the present application. The lamination of yarn layers 38 is stitched with a sewing yarn 39 and a shuttle yarn 40. The auxiliary needle 37 pierces the yarn layers 38 before the sewing needle 36, to facilitate the insertion of the sewing needle 36.

As the plurality of laminations of two-dimensional yarn layers are sewn together using the sewing machine, it is unnecessary to replace yarn guide pipes or pins with the coupling yarn. The fabric materials that are used in a reinforcing matrix are glass fiber, carbon fiber, ceramic fiber and the like, which do not stretch very much, and which are generally fragile. At the time the auxiliary needle 37 pierces the dense fiber structure, the needle 37 is likely to damage part of the fiber structure. In addition, it is difficult to secure sufficient space for the sewing needle 36 with the sewing yarn 39 inserted through its eye, to be smoothly inserted into the space formed by the auxiliary needle 37. Thus, when the sewing needle 36 pierces the fiber structure, it is likely to damage the fiber structure again.

Another method of producing a three-dimensional fabric has also been used. In this method, the yarn is placed between regulating members (pins) arranged at predetermined pitches on the base, and is looped back at the edges of the base, forming a lamination. The pins are replaced with vertical yarns using replacing members which hold coupling yarns (vertical yarns). In this case, the pins and the yarn lamination are removed from the base before the replacement operation. Then, the replacing member is placed on the associated pin and is pressed to drive out the pin and, at the same time, to insert the vertical yarn into the space formed by the pin. When the pins are removed from the base, however, both ends of each pin become free, so that the pins could tilt under the pressure of the laminated yarn layers. At this time, positions of the tips of the pins are not stable, thus making it difficult to mechanically abut the replacing members on the pins. It is therefore difficult to perform automatic replacement with a machine without misplacement of the vertical yarn.

#### SUMMARY OF THE INVENTION

Accordingly, it is a primary objective of the present invention to provide a method of producing a reinforcing matrix for a composite, which allows the yarn holding a lamination from both the front and back sides, to significantly reduce periodic lifting of the yarn lamination, thereby enhancing the fiber filling factor, and preventing a variation in the vertical and longitudinal dimensions.

It is another objective of the present invention to provide a method of producing a reinforcing matrix for a composite, which allows vertical yarns to be easily and securely inserted into spaces formed by regulating members or pins, for interconnecting the yarn layers.

To achieve the first objective, a reinforcing matrix for a composite according to the present invention uses a base on which a number of pins project upwardly, and are removably provided upright, in a plurality of rows, at predetermined pitches, along one predetermined direction. The reinforcing matrix is produced by the following methods:

(1) Weave yarns between the pins on the base, while repeatedly looping back at proper positions, to form a yarn lamination consisting of a plurality of yarn layers along the surface of the base. The yarns form yarn layers arranged in at least two directions.

(2) Remove the yarn lamination, formed on the base, together with the pins from the base.

5 (3) Sequentially replace the regulating members, arranged in a predetermined direction relative to the yarn lamination, with separate vertical yarns, which are inserted into the yarn lamination, and which form corresponding loops.

(4) Insert a selvage thread to be arranged in the predetermined direction of the yarn lamination into the loops of the vertical yarns.

The selvage thread is arranged in a predetermined direction of the yarn lamination, while the vertical yarns are arranged on the top surface of the yarn lamination in the direction perpendicular to the predetermined direction of the yarn lamination. Therefore, the vertical yarns and the selvage thread press the yarn lamination in the mutually perpendicular directions from both the front and back sides of the yarn lamination. This will prevent both the front and back surfaces of the yarn lamination from periodically expanding. It is therefore possible to enhance the fiber filling factor and to prevent variation of the vertical and longitudinal dimensions.

Another method of producing a three-dimensional fabric has also been used. In this method, the yarn is placed between regulating members (pins) arranged at predetermined pitches on the base, and is looped back at the edges of the base, forming a lamination. The pins are replaced with vertical yarns using replacing members which hold coupling yarns (vertical yarns). In this case, the pins and the yarn lamination are removed from the base before the replacement operation. Then, the replacing member is placed on the associated pin and is pressed to drive out the pin and, at the same time, to insert the vertical yarn into the space formed by the pin. When the pins are removed from the base, however, both ends of each pin become free, so that the pins could tilt under the pressure of the laminated yarn layers. At this time, positions of the tips of the pins are not stable, thus making it difficult to mechanically abut the replacing members on the pins. It is therefore difficult to perform automatic replacement with a machine without misplacement of the vertical yarn.

The spaces are formed by the pins at predetermined positions in association with the position of arrangement of the yarn lamination. Therefore, the step of positioning the yarn inserting members in the spaces is relatively easier than the step of abutting the yarn inserting members on the tips of the pins. The spaces formed by the removal of the pins are equal to, or slightly smaller than the diameter of the pins. This allows the yarn inserting members to be placed into the yarn lamination with slight contact therewith, so that the pins can be replaced with the vertical yarns without causing significant damage to the yarn lamination.

If the replacement of the pins with the vertical yarns is carried out according to the following two steps, a plurality of pins can be simultaneously replaced with vertical yarns, thus improving productivity:

(1) With the vertical yarns retained by the yarn inserting members corresponding in number to the pins which are arranged in one predetermined direction of the yarn lamination, the yarn inserting members are replaced with the pins, and the regulating members are simultaneously inserted into the lamination, until those portions of the yarn inserting members that are holding the vertical yarns come out of the yarn lamination.

(2) A selvage thread is inserted into the loops of the respective vertical yarns held by the yarn inserting members, in the direction of arrangement of the yarn inserting members, and then the yarn inserting members are pulled back to their original positions.

#### BRIEF DESCRIPTION OF THE DRAWINGS

The features of the present invention that are believed to be novel are set forth with particularity in the appended claims. The invention, together with objects and advantages thereof, may best be understood by reference to the following description of the presently preferred embodiments together with the accompanying drawings, in which:

FIG. 1 is a schematic perspective view showing a base used in producing a reinforcing matrix for a composite, according to a first embodiment of the present invention;

FIG. 2 is a schematic perspective view illustrating the arrangement of a plurality of support plates, a yarn lamination, and a plurality of pressure plates on the base shown in FIG. 1;

FIG. 3 is a schematic plan view showing how a first yarn or weft (arranged in a first plane) is arranged on the base of FIG. 1;

FIG. 4 is a schematic plan view showing how a second yarn or warp (arranged in a second plane) is arranged on the base of FIG. 1;

FIG. 5 is a schematic plan view showing how a first bias yarn is arranged on the base in FIG. 1;

FIG. 6 is a schematic plan view showing how a second bias yarn is arranged on the base in FIG. 1;

FIG. 7 is a schematic perspective view showing the positional relationship between the yarn lamination, and a first set of needles, when a plurality of pins are replaced with vertical yarns;

FIG. 8 is a schematic perspective view illustrating the set of first needles at positions corresponding to a second row of the pins;

FIG. 9 is a schematic perspective view illustrating the first set of needles abutting the pins;

FIG. 10 is a schematic perspective view showing the first set of needles inserted into the yarn lamination;

FIG. 11 is a schematic perspective view showing a second needle inserted through the loops of the vertical yarns;

FIG. 12 is a schematic perspective view showing a selvage thread inserted through the loops of the vertical 35 yarns;

FIG. 13 is a schematic perspective view illustrating the first set of needles pulled back to the original positions;

FIG. 14 is a schematic bottom view of the lamination, corresponding to FIG. 10;

FIG. 15 is a schematic bottom view of the lamination, corresponding to FIG. 11;

FIG. 16 is a schematic bottom view of the lamination, corresponding to FIG. 12;

FIG. 17 is an exemplary cross sectional view of a reinforcing matrix;

FIG. 18 is a schematic perspective view after the replacement of a second row of pins with vertical yarns, has been completed, according to a second embodiment of the present invention;

FIG. 19 is a schematic perspective view of the yarn lamination, after a third row of pins have been removed;

FIG. 20 is a schematic perspective view showing the first needles inserted into the yarn lamination;

FIG. 21 is an exemplary cross section showing the relationship between a base, pins, support plates, and pressure plates according to a third embodiment of the present invention;

FIGS. 22 through 28 are exemplary cross sectional views illustrating the steps of replacing the pins with vertical yarns in the third embodiment;

FIG. 29 is an exemplary cross sectional view illustrating the step of replacing yarn guide pipes with lines of 65 endless yarn according to the prior art; and

FIG. 30 is a schematic perspective view showing another embodiment according to the prior art.

## DETAILED DESCRIPTION OF THE PREFERRED EMBODIMENTS

### First Embodiment

A first embodiment of the present invention includes a method for producing a flat reinforcing matrix for a composite, and will now be described referring to FIGS. 1 through 17.

FIG. 1 shows a flat base 1, used in producing a reinforcing matrix. A plurality of pins 2 extend upwardly from one side of the base 1. The pins are disposed in a plurality of rows, that are placed at predetermined pitches along the width of the base 1. The pins 2 serve as regulating members to regulate the arrangement of the yarns. A plurality of support plates 3 are disposed on the base 1, between the pins 2. On the support plates 3, a first yarn or weft x is arranged in a first plane; a second yarn or warp y is arranged in a second plane; a first bias yarn B<sub>1</sub> and a second bias yarn B<sub>2</sub> are woven between the pins 2, and are repeatedly looped back and forth in engagement with the outer surfaces of the pins 2 which are located at the peripheral edges of the base 1, as shown in FIGS. 3 to 6. The weft layer x, warp layer y and bias-yarn layers B<sub>1</sub> and B<sub>2</sub> are laminated in a predetermined order.

As shown in FIG. 3, the lines of the weft x are arranged in parallel, along the width of the base 1, and are repeatedly looped back and forth around the pins 2 located at the corresponding opposite ends of the base 1. As shown in FIG. 4, the lines of the warp y are arranged in parallel along the length of the base 1, and are repeatedly looped back and forth around the pins 2 located at the corresponding opposite ends of the base 1. The lines of the first bias yarn B<sub>1</sub>, which form the first layer of a pair of bias-yarn layers, are arranged at an angle of +45° with respect to the length of the base 1, and are looped back and forth around the pins 2 located along the edges of the base 1, as shown in FIG. 5. The lines of the second bias yarn B<sub>2</sub>, which form the second layer of the bias-yarn layers, are arranged at an angle of -45° with respect to the length of the base 1, and are looped back and forth around the pins 2 located along the edges of the base 1, as shown in FIG. 6. Various fiber materials, such as carbon fiber, ceramic fiber, glass fiber, and aramid fiber, could be used for each yarn.

After the individual yarn layers are laminated on the base 1 in a predetermined order, to form a yarn lamination 4, a compressive force is applied thereon, to increase the density of the fibers of the yarn lamination 4, and to adjust the thickness thereof. More specifically, pressure plates 5 are arranged in parallel on the lamination 4 in association with the support plates 3, so that the lamination 4 is compressed by the support plates 3 and the pressure plates 5, as shown in FIG. 2. It is preferable that this compression be performed, not only when the arrangements of the weft x, warp y and the first and second bias yarns B<sub>1</sub> and B<sub>2</sub> are all completed, but also periodically, while arranging those yarns. This will 60 decrease the variation in the fiber density, and increase the fiber density.

Next, the lamination 4 and the pins 2 are separated from the base 1. The support plates 3 facilitate the separation of the pins 2 and the layer lamination 4 from the base 1. It is preferable that the weft x, warp y and both bias yarns B<sub>1</sub> and B<sub>2</sub> be arranged in a mirror symmetric fashion with respect to an imaginary plane at the center of the lamination 4, in the thickness or vertical direc-

tion, in order to prevent the reinforcing matrix from deforming after being impregnated with a resin.

The pins 2 are still placed into the lamination 4 after the separation from the base 1, and are replaced with vertical yarns z, such that the laminated layers are interconnected with the vertical yarns z. Unlike the prior art, one row of pins 2 arranged along the width of the lamination 4 are replaced with vertical yarns z simultaneously.

As shown in FIG. 7, a first set of needles 6 serves as yarn inserting members. The number of needles 6 is equal to the number of pins 2 arranged along the width direction of the lamination 4. The needles 6 are disposed at the same pitches as the pins 2. The first set of needles 6 have substantially the same diameter as that of the pins 2. The first set of needles 6 are arranged to be simultaneously moved up and down by a lifting mechanism (not shown). The vertical yarns z are fed out from a vertical-yarn feeding section (not shown). A tension adjuster 7 is provided between the vertical-yarn feeding section and the first set of needles 6, to absorb the slack of each vertical yarn z, and to apply tension to the yarn z.

The lamination 4 is supported by a supporting device (not shown) while being held by the support plates 3 and pressure plates 5. The supporting device can move the lamination 4 along a direction perpendicular to the direction of arrangement of the first set of needles 6. As one row of pins 2 is replaced with the vertical yarns z, the lamination 4 is moved in the direction of the arrow shown in FIG. 7, so that the next row of pins 2 face the first set of needles 6.

The replacement of the pins 2 with the vertical yarns z will be described in more detail referring to FIGS. 8 through 16. For convenience, the number of pins 2 and first set of needles 6 has been reduced, and the support plates 3 and pressure plates 5 have not been illustrated.

FIG. 8 illustrates the lamination 4 after replacement of two rows of pins 2 with the vertical yarns z. As illustrated in FIG. 9, the first set of needles 6 are simultaneously moved down, with their tips abutting the top portions of the pins 2. The first set of needles 6 are moved further down into the lamination 4, until eyes 6a holding the vertical yarns z come out on the bottom of the lamination 4 (see FIGS. 10 and 14). As a result, the pins 2 corresponding to the first set of needles 6 are driven out and the vertical yarns z are collectively inserted into the drive out spaces of the pins 2. Each vertical yarn forms a loop (L).

Next, as shown in FIG. 11, a second needle 8 is inserted through a loop LP of a lacking a selvage thread P that has previously been inserted in a single pass through the loops L of the vertical yarns z, and is moved forward in the direction of arrangement of the first set of needles 6. The tip of the second needle 8 sequentially passes through the loops L of the individual vertical yarns z, held by the respective first set of needles 6, and the second needle 8 stops when its tip reaches the edge of the lamination 4. At this time, the selvage thread P, fed out from a selvage-thread feeding section, comes in engagement with the tip of the second needle 8 (see FIG. 15).

A latch (not shown) of the second needle 8, disposed at the distal end thereof, is closed to prevent the loop L from being pulling back. The second needle 8 is then pulled back so that the selvage thread P is inserted, in a loop (LP), through the loops L of the vertical yarns z, as shown in FIG. 16. The loop LP of the selvage thread

P is held through the loop LP of the previous selvage thread P (see FIG. 12). Then, the first set of needles 6 is lifted up out of the lamination 4 to its original position. The vertical yarns z are pulled by the action of the tension adjuster 7 so as to tighten the vertical yarns z, which are retained by the selvage thread P (see FIG. 13).

The yarn lamination 4 is then moved to where the next row of pins 2 face the corresponding first act of needles 6. Then, one support plate 3 and one pressure plate 5 are removed, and the foregoing steps are repeated. In this manner, the pins 2 are sequentially replaced row by row with the vertical yarns z. Accordingly, the individual yarn layers, which form the lamination 4, are interconnected by the vertical yarns z, thus yielding a reinforcing matrix.

As mentioned earlier, the selvage thread P is arranged along the width direction of the lamination 4, while the vertical yarns z are arranged on the front side 10 of the lamination 4, along a direction that is perpendicular to the direction of arrangement of the selvage thread P. Therefore, the vertical yarns z and the selvage thread P press the lamination 4 along two perpendicular directions, from the front and back sides of the lamination 4. 20 Contrary to the case where the vertical yarns z and the selvage thread P are arranged in the same direction, both the front and back sides of the lamination 4 are prevented from developing periodic undulation extending in the same direction. Therefore, the fiber filling factor becomes uniform and increases. In addition, a variation of the width dimension of the yarn lamination 4 can be prevented. In impregnating the reinforcing matrix with a resin, therefore, uniform products composed of the matrix and the resin will be acquired without pressing the reinforcing matrix while stretching it.

The direction of arrangement of the vertical yarns z on the top surface of the lamination 4 differs from that of the selvage thread P. As shown in FIG. 17, the reinforcing matrix 9 is not symmetrical with respect to an imaginary plane passing through the center of the reinforcing matrix 9 in the thickness direction. Normally, the number of the vertical yarns z and the selvage thread P, including those present in the thickness (vertical) direction of the reinforcing matrix, as well as those 40 on the top and bottom surfaces thereof, is about 10% or less of the total amount of fibers that constitute the reinforcing matrix. The asymmetry of the arrangement of the vertical yarns z and selvage thread P will not therefore cause "deformation" after impregnation with a resin.

In addition, since, unlike in the prior art, the rows of pins 2 are replaced with the vertical yarns z, one row at a time, the production efficiency of the reinforcing matrix is improved.

## Second Embodiment

A second embodiment will now be described referring to FIGS. 18 to 20.

The method of producing a reinforcing matrix according to this embodiment is similar to that of the first embodiment up to the formation of the lamination 4. However, the step of replacing the pins 2 with the vertical yarns z, following the formation of the lamination 4 differs from that in the first embodiment. FIG. 18 illustrates the lamination 4 with two rows of pins 2 replaced with the vertical yarns z. Although not shown, the next row of pins 2 are pulled upward out of the lamination 4, without using the first set of needles 6, but with a Din

removing device (not shown). If the vertical yarns *z* extending from the tension adjuster 7 to the first set of needles 6 interfere with the pins 2, hindering the pin extraction, the pin extraction is performed after the lamination 4 is moved to where the obstruction does not occur. The materials for the individual yarns which constitute the lamination 4 are made of fibers with small extensibility, such as glass fiber, carbon fiber and ceramic fiber. The individual yarns remain at the previous positions for a while, even after the pins 2 are pulled out. Thus, the spaces formed in the lamination 4 by the extraction of the pins 2 therefrom, are almost equal to, or slightly smaller than the outside diameters of the pins 2.

Next, the lamination 4 is moved, so that spaces 4a face the first set of needles 6, as shown in FIG. 19. The drive-out spaces 4a are formed in the lamination 4 at the same pitches as the pitches of the pins 2 on the base 1 (not shown). By moving the lamination 4 to a predetermined position, therefore, the first set of needles 6 will be set facing the corresponding spaces 4a, easily and accurately. The first set of needles 6 is then simultaneously moved down, and inserted into the spaces 4a until the eyes 6a holding the vertical yarns *z* come out of the bottom of the lamination 4 (see FIG. 20). As a result, the vertical yarns *z* are inserted, each in a loop, into the lamination 4, where the removed pins 2 were located. Since the first set of needles 6 are placed into the spaces 4a, the first set of needles 6 will be inserted into the lamination 4 in slight contact therewith, and will not significantly damage the yarn lamination 4.

Then, as in the first embodiment, the selvage thread *P* is inserted, in a loop, through the loops *L* of the vertical yarns *z*. The first set of needles 6 is then lifted up out of the yarn lamination 4 to its original position. Then, the vertical yarns *z* are pulled by the action of the tension adjuster 7, so as to tighten the vertical yarns *z*, while the vertical yarns *z* are retained by the selvage thread *P*. Thereafter, the same process will be repeated and the pins 2 will be replaced, row by row, with the vertical *z* yarns *z*, for yielding a reinforcing matrix.

In this embodiment, the first set of needles 6 are placed into the spaces 4a, to insert the vertical yarns *z* into the lamination 4, thus ensuring easier positioning of the first set of needles 6 at the respective inserting positions as compared with the case where the first set of needles 6 are inserted into the lamination 4 while driving out the pins 2. This prevents the vertical yarns *z* from being inaccurately inserted. Further, as the extraction of the pins 2 and the insertion of the first set of needles 6 are performed independently, the necessary working spaces can be secured without substantial restriction on the size and shape of the reinforcing matrix. Therefore, the replacement can easily be automated.

### Third Embodiment

A third embodiment will now be described referring to FIGS. 21 through 28. In this embodiment, a reinforcing matrix having a U-shaped cross section, rather than a flat reinforcing matrix, is produced. As shown in FIG. 21, the base 1 is formed thicker than those of the previous embodiments, with a first end portion having a semicircular shape. The pins 2 are removably inserted at predetermined pitches, on the top and bottom surfaces of the base 1 and on the arcuate surface which is integral with the top and bottom surfaces of the base 1. The support plates 3 are disposed between the pins 2 along the width direction of the base 1 (the vertical

direction with respect to the plan of FIG. 21). As in the previous embodiments, the first and second bias yarns *B*<sub>1</sub> and *B*<sub>2</sub>, the weft *x*, and the warp *y*, are arranged so as to weave between the pins 2, and to be repeatedly looped back and forth in engagement with those pins 2 which are located along the edges of the base 1.

After the individual yarn layers are laminated in the predetermined order on the base 1, to yield the lamination 4, with a U-shaped cross section, the pressure plates 5 are disposed at the outer surface of the lamination 4. The pressure plates 5, formed into a U shape, are placed between the pins 2, perpendicularly to the support plates 3. After the lamination 4 is compressed by the support plates 3 and pressure plates 5, the lamination 4 and the pins 2 are separated from the base 1 (see FIG. 22).

Next, the pins 2, still inserted in the lamination 4, are replaced with the vertical yarns *z*, and the yarn layers of the lamination 4 are interconnected by the vertical yarns *z*. In this embodiment too, the rows of the pins 2 that are arranged along the width direction of the base 1 are replaced, row by row, with the vertical yarns. The lamination 4 is supported perpendicularly to the moving direction of the first set of needles 6 by a supporting device (not shown) while being held by the support plates 3 and pressure plates 5. The supporting device is designed in such a way that, at the position where the flat portions of the lamination 4 face the first set of needles 6, this device can move the yarn lamination 4 in a direction perpendicular to the direction of arrangement of the first set of needles 6. At the position where the curved portion of the lamination 4 faces the first set of needles 6, the supporting device can rotate the yarn lamination 4 around an axis, which passes through the center of curvature of the curved portion, and which extends in the direction of arrangement of the first set of needles 6.

FIG. 23 illustrates the lamination 4 moved to the position where the first set of needles 6 face the spaces 4a, formed by the extraction of the first row of pins 2 from the lamination 4. The pin extraction from the lamination 4 is carried out at the position where a pin removing device (not shown) does not interfere with the first set of needles 6 and vertical yarns. The first set of needles 6 are simultaneously moved down, and are inserted into the spaces 4a, until the eyes (not shown) of the first set of needles 6 come out of the bottom of the yarn lamination 4 (see FIG. 24). As a result, the vertical yarns *z* are inserted, each in a loop, into those portions of the lamination 4 where the pins 2 were located. Since the first set of needles 6 is placed into the spaces 4a, the first set of needles 6 will be inserted into the yarn lamination 4 in slight contact therewith, and will not significantly damage the yarn lamination 4.

Next, the second needle 8 is moved forward in the direction of arrangement of the first set of needles 6, and will stop when the tip of the second needle 8 passes through the loops *L* of the individual vertical yarns *m* held by the respective first set of needles 6, and reaches one end portion of the lamination 4. Then, the second needle 8 is pulled back so that the selvage thread *P* is inserted, in a loop, through the loops *L* of the vertical yarns *z*. Then, after the needles 6 are lifted out of the lamination 4 to their original positions, the vertical yarns *z* are pulled by the action of the tension adjuster 7 so as to tighten the vertical yarns *z*, while the vertical yarns *z* are retained by the selvage thread *P*. This com-

pletes the replacement of the first row of pins 2 with the vertical yarns z (see FIG. 15).

Then, after one support plate 3 is removed, the second row of pins 2 are pulled out, and the lamination 4 is moved to the position there the spaces &a face the first set of needles g (see FIG. 26). The needles 6 are then moved downward into the spaces 4a, and the second needle 8 is inserted through the loop portion (not shown) of the previous selvage thread P, and the loops L of the vertical yarns z, retained by the respective first set of needles 6 (see FIG. 27). After the selvage thread P, which is closer to the selvage-thread feeding section, is caught by the second needle 8, the second needle 8 is pulled back so that the selvage thread P is inserted through the loops L of the vertical yarns z.

The loop portion of the selvage thread P is held through the loop portion of the previous selvage thread P, similarly to the previous embodiments. After the loop portion of the previous selvage thread P is tightened, the needles 6 are lifted upwardly to their original positions. Then, the vertical yarns z, are tightened while being retained by the selvage thread P (see FIG. 28). Thereafter, the pins 2 are replaced in similar fashion, row by row, with the vertical yarns z, allowing the individual yarn layers of the lamination 4 to be interconnected with the vertical yarns z, for yielding a reinforcing matrix.

As the pins 2 are pulled out of the outer surface of the lamination 4, the resultant reinforcing matrix has a U shape with the two opposing faces, which will not hinder the pin extraction even if there is a small clearance between the opposing faces.

Although only three embodiments of the present invention have been described herein, it should be apparent to those skilled in the art that the present invention may be embodied in many other specific forms without departing from the spirit or scope of the invention. Particularly, it should be understood that this invention may be worked out in the following manners.

For instance, while the needles 6 have been described as being simultaneously inserted into the lamination 4, they could alternatively be separated into several groups such that they are inserted into the lamination 4 group by group. Alternatively, the needles 6 could be individually inserted, followed by the insertion of the vertical yarns s, the insertion of the selvage thread P, and the pulling of the vertical yarns z. Further, the regulating members or pins may be replaced, part by part, with the vertical yarns z using fewer needles 6 than regulating members (pins) arranged along the width direction. In this case, the pin extraction should be executed in synchronism with the timing of the insertion of the set of needles 6, for each pin targeted for the replacement.

Instead of the cylindrical pins 2, pipes or pins each having a recess at one end may be used as the regulating members. If pipes or pins each having a recess at one end are used in the first embodiment, the needles 6 would drive out the regulating members while in contact with the open ends of the pipes or the recesses of the pins, so that the needles 6 would securely engage the regulating members, thus ensuring smoother extraction.

Instead of repeating the insertion of the loop LP of the selvage thread P into the loop LP of the previous selvage thread P, the selvage thread P could be retained by simply stretching the vertical yarns z.

The replacement of the regulating members with the vertical yarns z may be performed for each line of regulating members arranged along the longitudinal direction of the lamination 4, instead of each row of regulating members arranged along the width direction. In this case, the selvage thread P runs along the longitudinal direction of the lamination 4, and the vertical yarns z on the top surface of the lamination 4 are arranged along the width direction of the lamination 4.

The inclination angle of the bias yarns B<sub>1</sub> and B<sub>2</sub>, which constitute the lamination 4, may be other than 45°. Instead of using both bias yarns B<sub>1</sub> and B<sub>2</sub>, the lamination 4 may consist of two types of yarn, the weft x and warp y, to provide a reinforcing matrix, which has a three-axis three-dimensional fiber structure. Further, the bias yarns B<sub>1</sub> and B<sub>2</sub> that form a pair of bias-yarn layers may be arranged with an inclination angle of 60° with respect to the warp y, while no weft x is used, thereby providing a reinforcing matrix which has a four-axis three-dimensional fiber structure. Furthermore, the order of the arrangement of the weft x, the warp y and the bias yarns B<sub>1</sub> and B<sub>2</sub> may be set arbitrarily, and the proper resin impregnation and proper fabric forming technology may be selected to prevent the deformation of the reinforcing matrix after the resin impregnation or the fabric formation is performed. Instead of using each single line of weft x, warp y and bias yarns B<sub>1</sub> and B<sub>2</sub> to form the respective yarn layers, each yarn layer may be formed of a plurality of lines of yarns.

The shape of the reinforcing matrix is not limited to a flat shape or a U shape, but may take other forms, such as an L shape or a box shape. The latter reinforcing matrix can be produced in the same manner as the former reinforcing matrix, using many pins or pipes extending upwardly from the base having an L shape, a box shape or some other shape.

In the case where the needles 6 are inserted into the spaces 4a, the pins 2 may be extracted from the yarn lamination 4, from the opposite side, to the needle inserting side, if such action does not interfere with the replacement process.

In addition, the regulating members while retaining the vertical yarns z may be pulled out of the lamination 4, and at the same time, the vertical yarns z may be inserted into the lamination 4 without using the needles 6. One way to accomplish this is to pull out the pins each having an engaging portion at the tip, from the lamination 4, while the vertical yarns z are engaged with the engaging portions of the pins. Another way is to use pipes as regulating members, form a suction air stream at one end of each pipe to suck and hold the vertical yarn z held in the vicinity of the other end of the pipe, and pull out the pipes in this condition out of the lamination 4. In either case, each of the vertical yarns z is inserted, in a loop, into the lamination 4, so that the loops protrude from the lamination 4.

Therefore, the present examples and embodiments are to be considered as illustrative and not restrictive and the invention is not to be limited to the details given herein, but may be modified within the scope of the appended claims.

What is claimed is:

1. A method of producing a reinforcing matrix for a composite, comprising the steps of:  
locating on a base a plurality of regulating members arranged in rows that extend in a first predetermined direction;

weaving yarns between said regulating members to form a lamination having a plurality of yarn layers on said base, said yarn layers having said yarns arranged in at least two different directions of said lamination; 5  
 simultaneously removing said lamination and said regulating members from said base; collectively forming a plurality of loops corresponding to said plurality of regulating members by collectively replacing said regulating members with a plurality of vertical yarns, each of said vertical 10  
 15  
 20  
 25  
 30  
 35  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990  
 5995  
 6000  
 6005  
 6010  
 6015  
 6020  
 6025  
 6030  
 6035  
 6040  
 6045  
 6050  
 6055  
 6060  
 6065  
 6070  
 6075  
 6080  
 6085  
 6090  
 6095  
 6100  
 6105  
 6110  
 6115  
 6120  
 6125  
 6130  
 6135  
 6140  
 6145  
 6150  
 6155  
 6160  
 6165  
 6170  
 6175  
 6180  
 6185  
 6190  
 6195  
 6200  
 6205  
 6210  
 6215  
 6220  
 6225  
 6230  
 6235  
 6240  
 6245  
 6250  
 6255  
 6260  
 6265  
 6270  
 6275  
 6280  
 6285  
 6290  
 6295  
 6300  
 6305  
 6310  
 6315  
 6320  
 6325  
 6330  
 6335  
 6340  
 6345  
 6350  
 6355  
 6360  
 6365  
 6370  
 6375  
 6380  
 6385  
 6390  
 6395  
 6400  
 6405  
 6410  
 6415  
 6420  
 6425  
 6430  
 6435  
 6440  
 6445  
 6450  
 6455  
 6460  
 6465  
 6470  
 6475  
 6480  
 6485  
 6490  
 6495  
 6500  
 6505  
 6510  
 6515  
 6520  
 6525  
 6530  
 6535  
 6540  
 6545  
 6550  
 6555  
 6560  
 6565  
 6570  
 6575  
 6580  
 6585  
 6590  
 6595  
 6600  
 6605  
 6610  
 6615  
 6620  
 6625  
 6630  
 6635  
 6640  
 6645  
 6650  
 6655  
 6660  
 6665  
 6670  
 6675  
 6680  
 6685  
 6690  
 6695  
 6700  
 6705  
 6710  
 6715  
 6720  
 6725  
 6730  
 6735  
 6740  
 6745  
 6750  
 6755  
 6760  
 6765  
 6770  
 6775  
 6780  
 6785  
 6790  
 6795  
 6800  
 6805  
 6810  
 6815  
 6820  
 6825  
 6830  
 6835  
 6840  
 6845  
 6850  
 6855  
 6860  
 6865  
 6870  
 6875  
 6880  
 6885  
 6890  
 6895  
 6900  
 6905  
 6910  
 6915  
 6920  
 6925  
 6930  
 6935  
 6940  
 6945  
 6950  
 6955  
 6960  
 6965  
 6970  
 6975  
 6980  
 6985  
 6990  
 6995  
 7000  
 7005  
 7010  
 7015  
 7020  
 7025  
 7030  
 7035  
 7040  
 7045  
 7050  
 7055  
 7060  
 7065  
 7070  
 7075  
 7080  
 7085  
 7090  
 7095  
 7100  
 7105  
 7110  
 7115  
 7120  
 7125  
 7130  
 7135  
 7140  
 7145

UNITED STATES PATENT AND TRADEMARK OFFICE  
CERTIFICATE OF CORRECTION

PATENT NO. : 5,327,621  
DATED : July 12, 1994  
INVENTOR(S) : Y. Yasui et al

Page 1 of 2

It is certified that error appears in the above-identified patent and that said Letters Patent is hereby corrected as shown below:

Column 2, line 6, after "repeated" insert --for--.

Column 3, line 2, change "at" to read --of--.

Column 6, line 12, "ping" should read --pins--;  
line 19, "planes" should read "plane;"; line 22, "pine"  
should read --pins--.

Column 7, line 3, delete "are still placed into", insert  
--remain in--; line 12, "pans" should read --pins--;  
line 44, "on" should read --of--; line 51, "lacking" should  
read --locking or--; line 52, delete "in a single pass";  
line 66, after "inserted," insert --in a single pass,--.

Column 8, line 13, change "raw" to read --row--; line 67  
"pans" should read --pins--; line 68, "Din" should read  
--pin--.

Column 9, line 10, "pine" should read --pins--; line 24,  
"s" should read --z--; line 48 "pine" should read  
--pins--; line 63 "ping" should read --pins--; line 67 "pine"  
should read --pins--.

Column 10, line 23, after "by" insert --row,--; line 45, after  
"yarns" and before the period insert --z--; line 59,  
change "m" to --z--.

UNITED STATES PATENT AND TRADEMARK OFFICE  
**CERTIFICATE OF CORRECTION**

PATENT NO. : 5,327,621.  
DATED : July 12, 1994  
INVENTOR(S) : Y. Yasui et al

Page 2 of 2

It is certified that error appears in the above-identified patent and that said Letters Patent is hereby corrected as shown below:

Column 11, line 5 "&a" should read --4a--; line 6, "g" should read --6--; line 47, "s," should read --z,--.

Column 12, line 50, "pine." should read --pins.--

Column 13, line 17, start new line at "locating".

Column 14, line 1, "member" should read --members--.

Column 14, line 37, "laminations;" should read --lamination--.

Signed and Sealed this  
Tenth Day of January, 1995

Attest:



BRUCE LEHMAN

Attesting Officer

Commissioner of Patents and Trademarks